# EUROPEAN PATENT APPLICATION

(11) **EP 0 407 061 A1**
(43) Date of publication of application: **09.01.1991**
(21) Application number: 90306756.9
(22) Date of filing: 20.06.1990
(51) Int. Cl.: H01B 3/30, H01B 7/28

(54) **Wire insulation**

(30) Priority: 04.07.1989 GB 8915349; 04.08.1989 GB 8917904; 08.12.1989 GB 8927831
(71) Applicant: ASSOCIATED ELECTRICAL INDUSTRIES LIMITED, London W1A 1EH (GB)
(72) Inventor: Murphy, Richard John, Liverpool L4 0RA (GB)
(74) Representative: Wood, John Irwin (GB)

(57) **Abstract**

A wire having an inner coating of a highly-insulative, halogen-free plastics material and a halogen-free, hard, flexible outer coating of a copolymer of, or a mixture of, a siloxane and a polyetherimide. An improvement is possible by adding a layer of poly-ether-etherketone as a further outer coating over the flexible coating.

## Description

This invention relates to plastics insulated wires.

It has been found extremely difficult, if not impossible, to produce a wire insulation which contains no halogens, passes high temperature flammability tests, has a high mechanical strength, is sufficiently flexible to be viable as a wire insulation, and does not catastrophically allow arc tracking.

It is well known that highly aromatic polymers are relatively non-flammable and have, in general, a high mechanical strength. However, these materials are stiff, and render the wire insulation rigid, so that the coated wire becomes non-flexible and effectively non-usable in practice. They are usually susceptible to arc tracking because they have a highly aromatic nature.

Accordingly, the invention provides a wire having an inner coating of a highly-insulative, halogen-free plastics material and a halogen-free, hard, flexible outer coating of a copolymer of, or a mixture of, a siloxane and a polyetherimide.

The inner coating may be of any modified polyolefinic material which is halogen-free and which does not promote arc-tracking. It may be cross-linked by radiation but this is not necessary if a high temperature deformation resistance is inherent in the polymer, or is provided by some other means. Suitable materials, singly or in combination, are.. poly(ethylene vinyl acetate)-EVA or VAE; poly(ethylene); poly(butyleneteraphthalate)-PBT; a thermoplastic elastomer; and a cross-linked elastomer.

The outer coating is of low flammability and is preferably cross-linkable. The siloxane may be polydimethylsiloxane or another substituted siloxane, and a suitable copolymer of polydimethylsiloxane and polyetherimide is available from General Electric Plastics Company (of the U.S.A.) under the trademark "SILTEM". In addition, it is found that improved performance can be obtained by blending the "SILTEM" copolymer with such polymers as polyphenylene ether or nylon.

The insulation may be improved significantly by the addition of a layer of poly-ether-etherketone ("PEEK") over the two coatings mentioned above. The flammability is lowered, the resistance to cut-through and abrasion is raised, and the resistance to attack by fluid or gaseous chemicals is improved. It is found surprisingly that this additional layer of PEEK does not significantly reduce the flexibility or resistance to arc tracking afforded by the first two coatings.

### EXAMPLE

An electric wire was made by coating a conductor with an extruded inner layer of modified polyethylene and then an extruded outer layer of "SILTEM" copolymer. The coated wire was then subjected to electron beam irradiation for cross-linking to a dose of 8 Mrad. in one case, and to 10, 12 and 15 Mrad. in other cases. All wires satisfied tests for vertical flammability, scrape abrasion, flexibility, arc tracking, cut-through resistance and resistance to oils and water.

## Claims

1. A wire having an inner coating of a highly-insulative, halogen-free plastics material and a halogen-free, hard, flexible outer coating comprising a copolymer of, or a mixture of, a siloxane and a polyetherimide.

2. A wire according to Claim 1, in which the inner coating is of any modified polyolefinic material which is halogen-free and which does not promote arc-tracking.

3. A wire according to Claim 2, in which the inner coating is of one or more materials selected from. poly(ethylene vinyl acetate)-EVA or VAE, poly(ethylene); poly(butyleneteraphthalate)-PBT; a thermoplastic elastomer; and a cross-linked elastomer.

4. A wire according to Claim 1, 2 or 3, in which the siloxane is polydimethylsiloxane or another substituted siloxane.

5. A wire according to any preceding claim, in which the outer coating is comprised of a mixture of a copolymer of siloxane and polyetherimide and another polymer.

6. A wire according to Claim 5, in which the said other polymer is polyphenylene oxide.

7. A wire according to Claim 5, in which the said other polymer is nylon.

8. A wire according to any preceding claim, further comprising an outer layer of PEEK over the flexible outer coating.
